

3,514,249

**STRETCHABLE WOVEN FABRICS**

John W. Bullington, Athens, and John H. Gustafson and Julian J. Hirshfeld, Decatur, Ala., assignors to Monsanto Company, St. Louis, Mo., a corporation of Delaware

No Drawing, Filed Jan. 20, 1966, Ser. No. 521,813

Int. Cl. D06m 5/12, 9/12, 9/14

U.S. Cl. 8—130.1

10 Claims

**ABSTRACT OF THE DISCLOSURE**

Stretch characteristics are imparted to fabrics having filling yarns comprised of polyester fiber by contacting the fabric with a swelling agent, applying a tension force in the direction of the warp yarns of the fabric, and vaporizing the swelling agent while the fabric is under the tension force.

This invention relates to a novel process of imparting a stretch characteristic to fabrics having filling yarns comprised of polyester fibers. More particularly, the invention relates to a novel method of imparting a stretch characteristic with maximum stretch growth to fabrics having filling yarns comprised of polyester fibers.

Stretch fabrics have the capability to stretch when under tension and then to contract to their original dimension when the tension is released. Such a capability gives to articles made of these fabrics many improved characteristics, e.g. improves the appearance of the articles because the fabric can give with a strain and then assume its original shape when the strain is released; improves the comfort of articles (stretch characteristics permit the body to move with minimum restraint from stretch garments, thereby increasing comfort); improves the fullness or thickness of articles causing a pleasing illustration of lightness or featherness of hand; improves the drape of the articles; improves the crease retention of articles that are pressed with a crease; improves the wash and wear characteristics of fabrics that are utilized in wash and wear garments; and improves the sizing of the article (articles such as garments having a particular size can adapt to individual variations within that size). The degree of stretch which is capable of imparting the above characteristics to the articles is usually at least about 15% with a maximum of about 2.5% growth, i.e. the fabric will not dimensionally grow above 2.5% over its original dimension after repeated stretchings.

Stretch fabrics are particularly useful in the apparel wear. They have received popular use in shirts, slacks, jackets, shorts, skirts, uniforms, dresses, children's wear, lingerie, suits, sportswear, etc. The fabrics are also useful in domestic and home furnishings, for example in contour sheeting and mattress covers, drapes, upholstery, and numerous other items.

Most of the stretch fabrics on the market are fabrics woven from stretchable yarns. Such stretch yarns can be made by different, e.g. by twisting (either false or conventional twisting), by stuffer box or gear crimp methods, by heating the yarn and drawing it over a crimping edge and by entangling the yarn with a stream of gas. After the yarn is processed into a stretchable yarn, the stretch yarns are woven into a fabric to give a stretchable fabric. Such stretchable fabrics are expensive to make due to the processes of stretching the yarn and then weaving such yarns into a fabric.

Incorporating stretch characteristics into a fabric composed of yarns other than prestretched yarn is relatively new. Such can be accomplished by treating a fabric composed of crimp yarns with a resin and curing the resin while the fabric is in the relaxed state. This treatment

produces a fabric composed of resilient-like crimp yarns which will stretch and when the stretching force is released will spring back into their original shape. However such a treatment adversely affects the characteristics of the fabric, for example the softness and drape are adversely affected.

A limited degree of stretch can be incorporated into fabrics by warp tensioning a fabric composed of thermoplastic yarns, that is causing the warp yarns to straighten and the filling yarns to pucker, and simultaneously heat-setting the yarns in such a position which results in a fabric having a fill stretch with good recovery. However, such a stretch process requires a large tensioning force and gives a limited amount of stretch to the fabric, usually less than 10%.

It is an object of this invention to provide a process for incorporating a stretch characteristic to fabrics having filling yarns comprised of polyester fiber.

Another object of the invention is to provide a method of producing stretch fabrics having filling yarns comprised of polyester fiber which are capable of stretching at least about 15% with a maximum of about 2.5% growth in the direction of the filling yarns.

Still another object of the invention is to provide a fabric having filling yarns comprised of polyester fiber which are capable of stretching at least about 15% with less than 2.5% growth in the direction of the filling yarns.

These and other objects of this invention are accomplished by providing a process for imparting a stretch characteristic to a fabric having filling yarns comprised of polyester fiber comprising contacting the fabric with a swelling agent, applying a tension force in the direction of the warp yarns of the fabric, and vaporizing the swelling agent while the fabric is under the tension force. Stretch fabrics made by this process exhibit a minimum of 15% filling stretch with less than 2.5% growth even after repeated washings and stretchings.

The fabrics useful with the invention are woven fabrics having filling yarns comprised of polyester fiber. The filling yarns can also be defined as the woof or weft yarns. The warp yarns of the fabric can be of any fiber, examples of warp yarns include yarns composed of one or more of the below fibers. Examples of filling yarns comprised of polyester yarns useful with the invention include yarns composed of polyester fiber or polyesters fiber with one or more fibers selected from the group consisting of wool, cotton, silk, rayon fiber (a manufactured fiber composed of regenerated cellulose, as well as manufactured fibers composed of regenerated cellulose in which substituents have replaced not more than 15% of the hydrogens of the hydroxyl groups), acetate fiber (a manufactured fiber in which the fiber-forming substance is cellulose acetate; where not less than 92% of the hydroxyl groups are acetylated, the term tri-acetate may be used as a generic description of the fiber), acrylic fiber (a manufactured fiber in which the fiber-forming substance is any long-chain synthetic polymer composed of at least 85% by weight of acrylonitrile units), modacrylic fiber (a manufactured fiber in which the fiber-forming substance is any long-chain synthetic polymer composed of less than 85% but at least about 35% by weight of acrylonitrile units), olefin fiber (a manufactured fiber in which the fiber-forming substance is any long-chain synthetic polymer composed of at least 85% by weight of ethylene, propylene or other olefin units), fluorocarbon fiber (a fiber formed of long-chain carbon molecules wherein the available bonds are saturated with fluorine), polyamide fiber (a manufactured fiber in which the fiber-forming substance is any long-chain synthetic polyamide having recurring amide groups (—CO—NH—) as an integral part of the polymer chain), etc. A particularly useful fabric is a fabric containing filling yarns composed

of at least 50% polyester fiber and the remainder cotton fiber.

The term "polyester fiber," as used herein, is defined as a manufactured fiber in which the fiber-forming substance is any long-chain synthetic polymer composed of at least 85% by weight of an ester of a dihydric alcohol and a dicarboxylic acid and copolymers or modifications of these polyesters and copolymers. The polyesters and copolymers are those resulting from the polymerization of one or more of the glycols of the series,  $\text{HO}(\text{CH}_2)_n\text{OH}$ , in which  $n$  is an integer from about 2 to about 10, with one or more dicarboxylic acids as ester-forming derivatives thereof. Examples of useful polyester fibers can be found in U.S. 3,063,956. Particularly useful polyester fibers are those composed of the poly-condensation product of ethylene glycol and terephthalic acid, ethylene glycol and dimethylterephthalate, and ethylene glycol and other ester-forming derivatives of the terephthalic acid.

Construction of the fabric should be a woven construction. Also, the construction of the fabric should permit the yarns to have some degree of movement, i.e. an open type construction as opposed to a tightly woven construction is preferred. A plain weave construction permits optimum freedom of movement of the yarns which will give good stretch characteristics when used with the invention.

As mentioned previously, the fabrics useful with the invention include fabrics having filling yarns comprised of polyester yarns, for example the filling yarns can contain 100% polyester fiber or the filling yarns can be a blend of polyester fiber and one or more of the fibers selected from the group consisting of cotton, wool, silk, rayon, acetate, acrylic, modacrylic, olefin, fluorocarbon, polyamide, etc. The stretch characteristics incorporated into the fabrics of this invention is in the direction of the filling yarns. Where the filling yarn is a blend of fibers, it is preferred that at least 50% of the filling yarn be polyester fiber; the warp yarns of the fabric can be any of the herein enumerated yarns.

Swelling agents useful with the invention include any swelling agent which can impart a plasticizing and swelling characteristic to polyester fiber. Examples of useful swelling agents include o-phenylphenol, p-phenylphenol, diphenyl, methylphenylcarbinol, monochlorobenzene, benzoic acid, salicylic acid and methyl salicylate. Examples of commercially available swelling agents identified by tradenames include Carolid (a self-emulsifiable modified phenol derivative, Carolid ELF-C (a nonionic, modified biphenyl derivative, Kayron CP (a self-emulsifiable solvent-modified phenol carrier, and Cindy DAC-888 (a self-emulsifying blend of alkyl and aryl esters. From a cost basis, o-phenylphenol is a preferred swelling agent useful with the process of this invention. The most significant effect of the swelling agent on the fabrics of this invention occurs as the swelling agent is being vaporized.

The novel stretch characteristics of the invention are imparted to the fabric by contacting the fabric with a swelling agent, applying a tension force to the fabric in the direction of the warp yarns and then vaporizing the swelling agent while the fabric is under the tension force. Contacting the fabric with the swelling agent can be accomplished by immersion, spraying, kiss rolling, vapor, exhaust, etc. It is preferred that the method of contacting the fabric should accomplish a sufficient swelling-agent uptake on the fabric to plasticize the polyester fiber. The period of contact time and the temperature of the swelling agent can be varied to meet the requirements of the particular contact method. Contacting the fabric with a swelling agent at a temperature substantially above room temperature, e.g. 200° F., will facilitate the uptake of the swelling agent on the fabric. However, the temperature of the swelling agent and the period of contact time is not critical as long as the uptake of the swelling agent on the fabric is sufficient to plasticize the polyester fiber. For example, where the polyester fiber is Dacron 54, an E. I. du Pont product, a swelling agent uptake of about

0.25 to about 10% of o-phenylphenol, based on the fabric weight, is sufficient to plasticize the polyester fiber.

The tension force applied to the fabric should be applied in the direction of the warp yarns of the fabric and should be enough force to straighten the warp yarns and thus to crinkle or ripple the filling yarns or weft yarns. Generally a tension force within the range of from about 0.5 lb. per inch to about 6.0 lbs. per inch is sufficient to straighten the warp yarns and to crinkle or ripple the filling yarns; with a plain weave fabric a tension force of from about 0.5 lb. per inch to about 3 lbs. per inch is sufficient, however with a tighter woven fabric a tension force of from about 2 lbs. per inch up to about 4 lbs. per inch is useful. Vaporizing the swelling agent is accomplished while the fabric is under the tension force and is effected by subjecting the fabric to a temperature within the range of from about the vaporization temperature of the swelling agent up to the decomposition temperature or scorching temperature of the fabric. Examples of useful temperatures include temperatures within the range of from about 200° F. up to about 450° F., a temperature within the range of from about 320° F. up to about 425° F. is preferred. Temperatures effected by a dry heat are also preferred. After the swelling agent is vaporized, it is preferred that the fabric be cooled while under the tension force to a temperature of at least about 25° F. below the temperature at which the swelling agent is vaporized. This cooling is generally effected instantaneously by merely subjecting the tensioned fabric to a temperature substantially lower than the temperature at which the swelling agent is vaporized, for example at room temperature. Where the invention is practiced in a continuous process, a cooling period following the vaporization step is recommended. Such a cooling is necessary to set the filling yarns in their crinkle or ripple condition and, thus, give a fabric with a good stretch characteristic.

With the process of this invention, the amount of stretch imparted to the fabric is at least 15% in the direction of the filling yarns. However, a stretch characteristic of up to about 30% can also be obtained. After repeated stretchings, the fabric will not grow more than 2.5% in the stretch direction at a stretch level of 15% up to about 20%. The stretch fabrics of the invention have also the novelty of good dye uptake due to the presence of the swelling agent on the fabric. Stretch fabrics obtained by the process of this invention are particularly useful for fabrication into tailored garments where the stretch requirements are within the limits imparted by this process. Also, such stretch fabrics have the capability to maintain their stretch characteristics even after repeated washings, thus making them ideal for wash and wear garments.

Working examples are presented to illustrate the invention. The fabric samples used in the following examples are desized, scoured and dried. Desizing is effected by immersing the fabric in water for 5 minutes at 160° F., then adding to the water 3 cc. per liter of desizing and degumming agents such as Rapidase (defined as a standardized mixture containing amylolytic and proteolytic enzymes, marketed by Wallerstein Company, Division of Baxter Laboratories) and 0.5 cc. per liter of a non-ionic surfactant such as Sterox NJ (defined as alkylaryl polyoxyethylene ether, marketed by Monsanto Chemical Company) and maintaining the water mixture at 150° F. for 30 minutes, and thereafter rinsing the fabric sample in water for 5 minutes at 180° F. The fabric sample is then scoured by immersing the sample in an aqueous mixture at 200° F. for 4-5 minutes containing 3 grams per liter of sodium hydroxide, 6 grams per liter of mineral spirits, and 0.5 gram per liter of a non-ionic surfactant such as Sterox NJ; then adding 6 grams per liter of sodium bicarbonate to the aqueous mixture and maintaining the mixture at 140° F. for 20 minutes; and thereafter rinsing the sample with water. The fabric sample is dried at 225-250° F. in a loop dryer. Other chemicals of common knowledge to the art which are equivalent to the above chemicals can be substituted for those chemicals enumerated.

ated above, e.g. other nonionic surfactants can be substituted for Sterox NJ and other desizing and degumming agents can be substituted for Rapidase, etc.

After the fabric sample is desized, scoured, and dried it is cut into two pieces of 28" warp by 15" filling. A 1.5" sleeve is sewn into each warp end, the purpose of which is to support the fabric sample during the tensioning step. The above dimensions are not critical but were chosen on an arbitrary basis.

The tensioning step of the process used in each example is effected by inserting into each sleeve a steel rod, positioning one steel rod in a supporting position and attaching steel plates to the other rod to give the desired uniform tension in the warp direction of the fabric sample. The tension is measured in pounds per inch.

10 After the fabric samples are treated as described in the following examples, they are subjected to a stretch test to determine their stretch characteristics. Each sample is cut into three test strips, each strip measuring 2½" in the warp direction by the resulting dimension in the original 15" filling dimension, generally 12" to 14" due to the crinkling in the filling yarns. The 2½" warp is reduced to 2" by ravelling the filling yarns. The top of the strip is then clamped to the top of a vertical scale and a four pound weight is clamped to the other end of the strip. The strip is then exercised slowly three times between a zero load and the four pound load. Thereafter the strip is subjected to the four pound load and the stretched dimension of the strip is measured; this measurement in relation to the original dimension is used to calculate the percent stretch. The weight and clamp are then removed and after a 30 second rest period the dimension of the strip is measured; this measurement in relation to the original dimension determines the percent growth. This procedure is repeated on the three strips and the results are averaged to give the percent stretch and the percent growth for each sample.

15 The following examples are presented to illustrate the invention and are not to be construed as limitations thereof. Percents used are based on weight unless otherwise illustrated and tension of the fabric is always in the warp direction.

#### EXAMPLE I

20 A fabric sample containing warp and filling yarns of 65% polyester fiber (obtained from the polymerization of ethylene glycol and terephthalic acid) and 35% cotton fiber having a yarn number of 28/2-28/2 and a yarn count of 48 x 48 is put under a tension of 0.96 lb./in. and is immersed for 1 minute in a 212° F. aqueous mixture containing 10 grams per liter of o-phenylphenol. The sample is then removed and suspended under the same tension in a oven for 1 minute at 320° F. Thereafter the fabric sample is removed from the oven, permitted to cool momentarily at room temperature, the tension is released, and the sample is analyzed. The sample shows a 15.75% stretch and a 1.7% growth.

#### EXAMPLE II

25 A fabric sample described in Example I is treated as described in Example I. Analysis of the fabric shows a 18.25% stretch and a 2.1% growth.

#### EXAMPLE III

30 A fabric sample described in Example I is treated as in Example I except the oven temperature is at 392° F. Analysis of the sample shows a 17.6% stretch and a 2.5% growth.

#### EXAMPLE IV

35 A fabric sample described in Example I is treated as in Example I except the tension is 3.0 lb./in. and the oven temperature is 392° F. Analysis of the fabric sample shows a 18.55% stretch and a 2.5% growth.

#### EXAMPLE V

40 A fabric sample described in Example I is treated as in Example I except the tension is 0.53 lb./in. and the oven temperature is 284° F. Analysis of the fabric sample shows a 15.75% stretch and a 1.7% growth.

#### EXAMPLE VI

45 A fabric sample described in Example I is treated as in Example I except the tension is 1.95 lb./in. and the oven temperature is 284° F. Analysis of the fabric sample shows 18.35% stretch and 2.2% growth.

#### EXAMPLE VII

50 A fabric sample described in Example I is treated as in Example I except the tension is 0.53 lb./in. and the oven temperature is 356° F. Analysis of the sample shows a 16.10% stretch and a 2.1% growth.

#### EXAMPLE VIII

55 A fabric sample described in Example I is treated as in Example I except the tension is 0.95 lb./in. and the oven temperature is 356° F. Analysis of the sample shows a 17.35% stretch and a 2.1% growth.

#### EXAMPLE IX

60 A fabric sample described in Example I is treated as in Example I except the tension is 3.0 lb./in. and the oven temperature is 392° F. Analysis of the fabric sample shows 18.55% stretch and 2.5% growth.

#### EXAMPLE X

65 A 12 foot length fabric sample described in Example I is immersed for 1 minute in a 212° F. aqueous solution containing o-phenylphenol. The sample is then slowly pulled at a warp tension of 1.95 lb./in. through an oven maintained at 400° F. The rate of pull through the oven is at a rate such that the sample is dry as it leaves the oven. Analysis of the sample shows a 14.5% stretch and 0.7% growth.

#### EXAMPLE XI

70 To show the significance of the carrier and heat-set process over a heat-set process, the procedure in Example X is repeated on an identical fabric sample described in Example X except the sample is not immersed in an aqueous solution of o-phenylphenol. Analysis of the sample shows a 9.8% stretch and a 1.2% growth as compared to a 14.5% stretch and a 0.7% growth as indicated in Example X.

#### EXAMPLE XII

75 A woven fabric sample composed of warp and filling yarns being 60% polyester fiber and 40% cotton fiber and having a yarn number of 50/1 x 50/1 and a yarn count 72 x 72 is immersed for 1 minute in a boiling aqueous solution containing 10 grams per liter of o-phenylphenol. The sample is removed, 20.4 lb./in. in warp tension is applied and the tensioned fabric is suspended in a 400° F. oven for 2 minutes. The fabric is removed and analyzed. Analysis shows a 16.6% stretch and a 2.0% growth.

#### EXAMPLE XIII

80 A fabric sample composed of warp and filling yarns being 100% polyester fiber (obtained from spinning a polymer of ethylene glycol and terephthalic acid) is immersed for 1 minute in a 205° F. aqueous solution containing 10 grams per liter of o-phenylphenol. The fabric is then removed and a warp tension of 1.95 lb./in. is applied. The tensioned fabric is placed in an oven for 75 2 minutes at 400° F. The fabric is removed and analyzed.

Analysis of the fabric sample shows a 15.5% stretch and a 1.0% growth.

#### EXAMPLE XIV

A woven fabric composed of warp and filling yarns of 65% polyester fiber and 35% rayon fiber (Avril, trade name of American Viscose Corporation) and having a yarn count of 118 x 78 and weighing 3.7 ounces per square yard is immersed for 1 minute in a 205° F. aqueous solution containing 10 grams per liter of o-phenylphenol. The sample is removed, a warp tension of 2 lb./in. is applied and the tensioned fabric is placed in an oven for 2 minutes at 380° F. Thereafter, the sample is removed and analyzed. Analysis of the fabric shows a 15.0% stretch and a 2.0% growth and a yarn count of 136 x 70. The original yarn count of 116 x 72 as compared to 136 x 70, the yarn count of the treated fabric, indicates the change in character of the fabric sample due to the treatment.

#### EXAMPLE XV

A fabric sample composed of warp and filling yarns of 65% polyester fiber (obtained from spinning a polymer of ethylene glycol and dimethyl terephthalate) and 35% cotton fiber is immersed for 1 minute in a 205° F. aqueous solution containing 10 grams per liter of o-phenylphenol. The sample is removed, a 2.0 lb./in. warp tension is applied and the tensioned fabric sample is suspended in an oven maintained at 264° F. and kept in the oven for 2 minutes after the aqueous solution starts to vaporize. Thereafter the sample is removed and analyzed. Analysis of the fabric sample shows a 17.5% stretch and a 1.8% growth. The sample is then laundered and again analyzed. The laundered fabric sample shows a 17.0% stretch and a 2.0% growth.

#### EXAMPLE XVI

A fabric sample described in Example XV is treated as described in Example XV except the oven temperature is maintained at 318° F. Analysis of the sample shows a 19.0% stretch and 1.5% growth. After laundering the sample shows a 19.0% stretch and a 2.0% growth.

#### EXAMPLE XVII

A fabric sample described in Example XV is treated as described in Example XV except the oven temperature is maintained at 370° F. Analysis of the fabric sample shows a 18.2% stretch and 2.5% growth. After laundering, the fabric sample shows a 19.5% stretch and a 2.0% growth.

#### EXAMPLE XVIII

A fabric sample described in Example XV is treated as in Example XV except the oven temperature is maintained at 378° F. The fabric sample shows a 19.3% stretch and a 2.2% growth. After laundering the fabric sample shows a 20.7% stretch and a 2.0% growth.

#### EXAMPLE XIX

A fabric sample described in Example XV is treated as described in Example XV except the oven is maintained at 421° F. The fabric sample shows a 17.3% stretch and 1.3% growth. After laundering the fabric sample shows a 19.3% stretch and a 1.4% growth.

#### EXAMPLE XX

A fabric sample described in Example XV is treated as in Example XV except the oven is maintained at 266° F. The fabric sample shows a 19.5% stretch and a 1.2% growth. After laundering the fabric sample shows a 18.2% stretch and a 2.0% growth.

#### EXAMPLE XXI

A fabric sample described in Example XV is treated as in Example XV except the oven is maintained at 322°

F. Analysis of the fabric sample shows a 20.3% stretch and a 1.7% growth. After laundering the fabric sample shows a 20.5% stretch and a 2.5% growth.

#### EXAMPLE XXII

A fabric sample described in Example XV is treated as in Example XV except the oven temperature is maintained at 426° F. Analysis of the fabric sample shows a 15.3% stretch and a 1.5% growth. After laundering the fabric sample shows a 17.3% stretch and a 1.0% growth.

The above examples are presented to illustrate the invention and are not to be considered as a limitation thereof.

What is claimed is:

1. A process for imparting a stretch characteristic to a fabric having filling yarns comprised of at least 50% polyester fiber, consisting essentially of contacting the fabric with a swelling agent for polyester fibers, thereby plasticizing the polyester fibers, then applying a tension force of from about 0.5 lb. per inch to about 6.0 lbs. per inch to the fabric in the direction of the warp yarns in the fabric, vaporizing at a temperature within the range of from about the vaporization temperature of the swelling agent to about 450° F. the swelling agent while the fabric is under the tension force, and cooling the fabric while under the tension force to a temperature of at least about 25° F. below the temperature at which the swelling agent is vaporized.
2. The process of claim 1 wherein the filling yarns are composed of polyester fiber and cotton fiber.
3. The process of claim 1 wherein the filling yarns are composed of polyester fiber and wool fiber.
4. The process of claim 1 wherein the filling yarns are composed of polyester fiber and rayon fiber.
5. The process of claim 1 wherein the swelling agent is o-phenylphenol.
6. The process of claim 1 wherein the swelling agent is vaporized at a temperature within the range of from about 300° F. to about 425° F.
7. A fabric composed of filling yarns comprised of polyester fiber having a stretch characteristic in the direction of the filling yarns of the fabric obtained by a process which consists essentially of contacting the fabric with a swelling agent for polyester fibers, thereby plasticizing the polyester fibers, then applying a tension force of from about 0.5 lb. per inch to about 6 lbs. per inch to the fabric in the direction of the warp yarns in the fabric and vaporizing by heating at a temperature within the range of from about the vaporization temperature of the swelling agent to about 450° F. the swelling agent while the fabric is under the tension force, and cooling the fabric while under the tension force to a temperature of at least about 25° F. below the temperature at which the swelling agent is vaporized.
8. A fabric composed of filling yarns comprised of at least about 50% polyester fiber having a stretch characteristic of at least about 15% in the direction of the filling yarns of the fabric obtained by a process which consists essentially of contacting the fabric with a swelling agent for polyester fibers, thereby plasticizing the polyester fibers, then applying a tension force of from about 0.5 lb. per inch to about 6.0 lbs. per inch to the fabric in the direction of the warp yarns of the fabric, vaporizing a temperature within the range of from about the vaporization temperature of the swelling agent to about 450° F. the swelling agent while the fabric is under the tension force, and cooling the fabric while under the tension force to a temperature of at least about 25° F. below the temperature at which the swelling agent is vaporized.
9. The fabric of claim 8 wherein the fabric is composed of filling yarns being a blend of about 65% polyester fiber and about 35% cotton fiber.

10. The fabric of claim 8 wherein the fabric is composed of filling yarns being a blend of about 65% polyester fiber and about 35% rayon fiber.

**References Cited**

**UNITED STATES PATENTS**

2,404,837 7/1946 Goldthwait.  
 2,897,042 7/1959 Heiks ----- 8—130.1  
 3,290,752 12/1966 Ormand ----- 8—130.1 X

5 American Dyestuff Reporter, Jan. 20, 1964, p. 47(62),  
 heat setting of polyester fibers.

5 Canadian Textile Journal, vol. 81, No. 6, Mar. 13, 1964,  
 pp. 41—50, "Process and Properties of Cotton Stretch  
 Fabrics."

10 LEON D. ROSDOL, Primary Examiner  
 M. HALPERN, Assistant Examiner

**U.S. Cl. X.R.**

FOREIGN PATENTS  
 691,559 7/1964 Canada.

8—132, 1145

**OTHER REFERENCES**

American Dyestuff Reporter, Jan. 20, 1964, p. 47(62),  
 heat setting of polyester fibers.

Canadian Textile Journal, vol. 81, No. 6, Mar. 13, 1964,  
 pp. 41—50, "Process and Properties of Cotton Stretch  
 Fabrics."